

1

2,933,382

## JET FUEL COMPOSITIONS

Frederick M. Fowkes, Orinda, Calif., and Francis G. Bollo, Alton, Ill., assignors to Shell Oil Company, a corporation of Delaware

No Drawing. Application May 6, 1957  
Serial No. 657,041

6 Claims. (Cl. 52—5)

This invention relates to hydrocarbon fuels, particularly 15 to so-called jet fuels for use in jet aircraft engines.

2

carbons, containing only carbon and fluorine and may be obtained by completely fluorinating a light hydrocarbon distillate fraction, such as a fraction in the kerosene and/or light lubricating oil distillate range. Preferably the hydrocarbon material to be fluorinated should contain only a minor amount of aromatic and/or alicyclic hydrocarbons, i.e., it should be composed predominately of aliphatic, open-chain hydrocarbons.

Typical perfluorocarbons which are useful in the practice of the invention are set forth in Table I.

Perfluorocarbons such as composition F (Table I) or fractions thereof, such as fractions F<sub>1</sub>, F<sub>2</sub>, F<sub>3</sub>, F<sub>4</sub>, and F<sub>5</sub> (Table I) are suitable foam inhibitors for hydrocarbon jet fuels. They are essentially aliphatic compounds which contain carbon atoms arranged in a normal (straight-chain) or branched chain-structure.

TABLE I  
*Properties of various perfluorocarbons*

| Description                 | Empirical Formula                 | Identifi-<br>cation<br>Symbol | Mole-<br>cular<br>Weight<br>(approx.) | Boiling Point, °C.<br>(approx.) | Density<br>20° C.<br>(approx.) | Index of<br>Refrac-<br>tion<br>(approx.) | Solubility, wt.<br>Percent at 27° C. |                    | Benzene |
|-----------------------------|-----------------------------------|-------------------------------|---------------------------------------|---------------------------------|--------------------------------|------------------------------------------|--------------------------------------|--------------------|---------|
|                             |                                   |                               |                                       |                                 |                                |                                          | CCl <sub>4</sub>                     | CH <sub>3</sub> OH |         |
| Perfluorokerosene (FCX-329) | C <sub>12</sub> F <sub>29</sub>   | C                             | 645                                   | 20-65 at 10 mm. Hg              | 1.922                          | 1.3082                                   | <1                                   | <1                 | <1      |
| Perfluorokerosene (FCX-30)  | C <sub>11</sub> F <sub>29</sub>   | D                             | 738                                   | 65-130 at 10 mm. Hg             | 1.994                          | 1.3171                                   | <1                                   | <1                 | <1      |
| Perfluorolube oil (FCX-512) | C <sub>20</sub> F <sub>42</sub>   | E                             | 1,038                                 | 70-240 at 10 mm. Hg             | 2.059                          | 1.3369                                   | 3.4                                  | <1                 | <1      |
| Perfluorolube oil (FCX-412) | C <sub>21</sub> F <sub>44</sub> * | F                             | 1,126                                 | 130-240 at 10 mm. Hg            | —                              | 1.3430                                   | 2.7                                  | <1                 | <1      |

\* This material may be further fractionated into 5 different fractions having the following boiling point ranges at 10 mm. Hg abs. pressure and identified as:

|                                 |         |
|---------------------------------|---------|
| F <sub>1</sub> —Fraction No. 1. | 130-150 |
| F <sub>2</sub> —Fraction No. 2. | 150-170 |
| F <sub>3</sub> —Fraction No. 3. | 170-190 |
| F <sub>4</sub> —Fraction No. 4. | 190-210 |
| F <sub>5</sub> —Fraction No. 5. | 210-240 |

In our copending application, Serial No. 560,867, filed January 23, 1956, now abandoned, of which the present application is a continuation-in-part, it has been shown that conventional foam inhibitors such as silicone polymers are ineffective foam inhibitors for jet fuels, but that certain hydrocarbon-insoluble perfluorocarbons are effective foam inhibitors for jet fuels. However, the perfluorocarbon foam inhibitors tend to separate out of solution during storage. Therefore, caution must be taken to thoroughly mix stored fuels containing a perfluorocarbon foam inhibitor to redisperse it otherwise the fuel will not be sufficiently foam resistant.

Solubilization of the perfluorocarbon anti-foam agent in the jet fuel can be obtained by the use of solubilizers such as oil-soluble alcohols and oil-soluble amines, but they are unsuitable because they interfere with the foam inhibiting properties of the perfluorocarbons in the hydrocarbon fuel.

It has now been discovered that storage stable and improved foam resistant hydrocarbon jet fuels are provided by addition to the jet fuels of a minor amount of from about 0.0001% to about 1%, preferably from about 0.01% to about 0.1% by volume, of a hydrocarbon-insoluble perfluorocarbon (containing only carbon and fluorine) having at least 12 carbon atoms and mixtures thereof, and as anti-foam enhancers and emulsifiers for the perfluorocarbons, a minor amount of from about 0.01% to about 10%, preferably from about 0.1% to about 5%, of a polyfluoroamide containing a hydrocarbon-insoluble perfluorohydrocarbyl group and an oil-solubilizing aliphatic group in the molecule.

The perfluorocarbon foam inhibiting agents are prepared by the method described in the articles by Fowler et al. and Burford et al. in the March 1947 issue of Ind. and Eng. Chem. (vol. 39, No. 3, pages 292 and 319). The perfluorocarbons are essentially aliphatic perfluoro-

40 Mixtures of perfluorocarbons boiling above 130° C. at 10 mm. Hg pressure and having more than 12 carbon atoms with lower boiling perfluorocarbons (130° C. at atmos. pressure) or not less than 12 carbon atoms in the ratio of from 4:1 to 1:4, from 4:1 to 2:1 respectively, can be used. Thus mixtures of perfluorocarbons such as C and F or D and F (Table I) in the mole ratio of 1:4 respectively, can be used as the anti-foam inhibitors.

45 The polyfluoroamide anti-foam enhancing and emulsifying agents for the perfluorocarbon foam inhibitors in the jet fuel are suitably and readily prepared by reacting perfluorocarboxylic acid, preferably a perfluoroaliphatic monocarboxylic acid having from 4 to 22 (better 8 to 18) carbon atoms in the molecule with a hydrocarbon-soluble amine, preferably an aliphatic monoamine or an N-alkyl polymethylene diamine where the aliphatic radical contains from 8 to 22, preferably 12 to 18, carbon atoms. Also the perfluoroamide can be prepared by reacting an organic carboxylic acid preferably a hydrocarbon-soluble aliphatic monocarboxylic acid having from 8 to 18 carbon atoms in the molecule with a perfluoroalkylamine.

50 The perfluoro acids include perfluoro mono- and polycarboxylic acids. The C<sub>8</sub>-C<sub>18</sub> perfluoroaliphatic monocarboxylic acids are preferred. Examples of such acids are perfluorobutyric acid, perfluorocaproic acid, perfluorohexanoic acid, perfluorocaprylic acid, perfluorocapric acid, perfluorolauric acid, perfluorostearic acid and mixtures thereof. Other suitable perfluoroalkyl substituted carboxylic acids include perfluoroalkyl aryl carboxylic acids such as C<sub>4</sub>-C<sub>18</sub> perfluoroalkylbenzoic or salicylic acid; perfluoroalkyl substituted polycarboxylic acids such as perfluoroctyl, perfluorodecyl or perfluorododecyl succinic, adipic or sebatic acids.

55 Amines for use in amidizing the above acids include oil-soluble mono- or polyamines containing at least one alkyl radical of at least 8 carbon atoms. Monoamines

of this type include octyl, decyl, dodecyl, tetradecyl, hexadecyl and octadecyl monoamines. In the secondary amines the alkyl radicals can be the same or different. Aliphatic polyamines include N-alkyl substituted alkylenes polyamines wherein the alkylenes radical contains from 2 to 10 carbon atoms, such as N-alkyl substituted ethylene diamine, propylene diamine, butylene diamine, diethylene tetramine, tetraethylene pentamine and the alkyl substituent group(s) can be attached to the same or different nitrogen atoms in the molecule and should generally have from 8 to 22 carbon atoms. Preferred N-alkyl substituted methylene polyamines include N-C<sub>12-18</sub> alkyl trimethylene diamine, N-C<sub>17</sub>-alkyl trimethylene diamine, N-C<sub>18</sub>-alkyl trimethylene diamine, N-C<sub>11</sub> trimethylene diamine, and the like.

Also the above corresponding non-fluorinated acids such as C<sub>8</sub>-C<sub>18</sub> aliphatic monocarboxylic acids e.g., caprylic acid, lauric acid or stearic acid can be amidized with perfluoroalkylamines such as perfluoroctylamine, perfluorododecylamine, perfluoroctadecylamine, N-perfluoro C<sub>12-18</sub> alkyl trimethylene diamine and the like.

Examples of perfluoroamides are decyl perfluorocapryl amide, dodecyl perfluorocapryl amide, octadecyl perfluorocapryl amide, octyl perfluorolauryl amide, octalperfluorostearyl amide, N-C<sub>12-18</sub> alkyl trimethylene perfluorocapryl amide, octadecyl perfluorododecyladipyl amide, perfluoro-octyl capryl amide, perfluoro-octadecyl capryl amide, perfluorododecyl stearyl amide and mixtures thereof.

The jet fuels for aircrafts are commonly known by the JP-designation such as JP-1, JP-3, JP-4 or JP-5 under MIL-F-5624 B specification, the properties of which are given in Table II.

boil vigorously and to foam as a result thereof. It is considered that foaming is caused by the vigorous boiling of the jet fuel (due to its volatile low boiling constituents) in the presence of and/or aggravated by the presence of relatively high boiling hydrocarbons, e.g. those hydrocarbons boiling in the range of from about 450° F. to about 600° F. and higher. Accordingly, due to the presence of a greater amount of low boiling hydrocarbons, as evidenced by the higher Reid Vapor Pressure, and also due to the presence of a greater proportion of high boiling hydrocarbons, a JP-3 jet fuel boils and foams much more than a JP type of jet fuel. Jet fuels which have Reid Vapor Pressure between about 0.5 and about 10 lbs. per sq. in. at 100° F. and especially between about 15 2 and 7 lbs. per sq. in. are most susceptible to foam upon boiling and are advantageously improved in this respect, i.e., foaming is essentially eliminated by addition to such jet fuels (JP-3 fuels), of perfluorocarbons and are rendered storage stable by addition thereto of polyfluoroamides.

In order to demonstrate the effectiveness of compositions of this invention for their stability and resistance to foaming, a number of tests were carried out. The test apparatus for measuring foaming consisted of a long vertical 1½ inch diameter glass tube, representing a fuel tank, charged with 100 ml. of a representative type of jet fuel (JP-3). The air space above the test mixture was evacuated at a rate representative of the change in atmospheric pressure (ratio-of-climb performance) which would be experienced by a typical jet aircraft in a rapid climb. The foaming tendency was judged by the height of foam column produced in the tube above the fuel liquid.

TABLE III

[Base: JP-3 Fuel.]

| Foam Inhibitor                       | Per cent Vol. | Emulsifier                                                    | Per cent wt. | Height of Foam, in. | Separation Time |
|--------------------------------------|---------------|---------------------------------------------------------------|--------------|---------------------|-----------------|
| 1. None                              |               | None                                                          |              | 30                  |                 |
| 2. Dow Corning Silicone No. 200 a    | 0.02          | do                                                            |              | 29                  |                 |
| 3. Dow Corning Silicone No. 500      | 0.01          | do                                                            |              | 34                  |                 |
| 4. 1,3 bis (trifluoromethyl) benzene | 0.01          | do                                                            |              | 30                  | 2 hours.        |
| 5. Perfluorodimethylcyclohexane      | 0.1           | do                                                            |              | 28                  | Do.             |
| 6. Perfluorocaprylic acid            | 0.1           | do                                                            |              | 30                  | Do.             |
| 7. F <sub>1</sub> b                  | 0.02          | do                                                            |              | 2                   | Do.             |
| 8. F <sub>1</sub>                    | 0.02          | do                                                            |              | 3                   | Do.             |
| 9. F <sub>2</sub>                    | 0.02          | do                                                            |              | 3                   | Do.             |
| 10. F <sub>3</sub>                   | 0.02          | do                                                            |              | 3                   | Do.             |
| 11. F <sub>2</sub>                   |               | N-C <sub>12-18</sub> alkyl trimethylene perfluorocapryl amide | 0.5          | 30                  | 2 days.         |
| 12. F <sub>2</sub>                   |               | octadecylperfluorocapryl amide                                | 0.5          | 30                  | Do.             |
| 13. F <sub>2</sub>                   | 0.02          | N-C <sub>12-18</sub> alkyl trimethylene perfluorocapryl amide | 0.5          | 1                   | 5 days.         |
| 14. F <sub>1</sub>                   | 0.02          | N-C <sub>12-18</sub> alkyl trimethylene perfluorocapryl amide | 0.5          | 1                   | Do.             |
| 15. F <sub>2</sub>                   | 0.02          | octadecylperfluorocapryl amide                                | 0.5          | 3                   | Do.             |

a Dow Corning silicones are methyl silicone polymers described in the Jour. of Ind. Hygiene and Toxicology No. 1948, pp. 332-352 and in Dow Corning Bulletin entitled "New Engineering Materials DC Silicones" (1947).

b Note Table I for identification of compounds.

TABLE II

[MIL-F-5624 B.]

|                                      | JP-1  | JP-3  | JP-4  | JP-5  |
|--------------------------------------|-------|-------|-------|-------|
| Reid Vapor Pressure, lb. per sq. in. |       | 5-7   | 2-3   |       |
| ASTM Distillation:                   |       |       |       |       |
| 10% Distillation                     | 410   |       |       |       |
| 20% Evaporation at °F                |       | 240   | 270   |       |
| 90% Evaporation at °F                | 490   | 470   | 470   |       |
| End Point °F                         | 572   | 600   | 550   | 550   |
| Total Sulfur, Percent wt.            | 0.2   | 0.4   | 0.4   | 0.4   |
| Mercaptan sulfur, percent wt.        | 0.005 | 0.005 | 0.005 | 0.005 |
| Aromatics, vol. percent              | 20    | 25    | 25    | 25    |
| Freezing Point, °F                   | -76   | -76   | -76   | -40   |
| Gravity, API                         | 35    | 50-60 | 45-55 | 35-45 |

Jet fuels with the above characteristics upon being subjected to a rapid decrease in ambient pressure tend to

level. The stability was measured by noting the time it took for separation of the perfluorocarbon from the fuel compositions at room temperature. The results of the various tests are set forth in Table III.

From the above data it can be noted that conventional foam inhibitors such as silicone polymers (compositions 2 and 3) or certain fluorine-containing compounds (compositions 4-6) are ineffective as foam inhibitors in jet fuel and are unstable. Perfluorocarbons which are effective foam inhibitors are unstable separating out of the fuel (JP-3) in about 2 hours (compositions 7-10). The polyfluoroamides are ineffective as foam inhibitors, but the fuel containing them is storage stable (compositions 11 and 12). However, when the two additives are used together in the fuel, foaming is inhibited and the stability is greatly improved (compositions 13, 14 and 15). This

patent application is a continuation-in-part of copending patent application Serial No. 560,867, filed January 23, 1956, which is, in turn, a continuation-in-part of patent application Serial No. 204,834, filed January 6, 1951, now abandoned.

We claim as our invention:

1. A stable, non-foaming petroleum hydrocarbon jet fuel composition consisting essentially of a major amount of a petroleum hydrocarbon jet fuel having a boiling range from about 240° F. to about 600° F. and containing from about 0.001% to about 1% by volume of a hydrocarbon-insoluble saturated perfluorocarbon having from 12 to 21 carbon atoms and having a boiling point range of from about 20° C. to about 240° C. at 10 mm. Hg and from about 0.01% to about 10% of a hydrocarbon dispersible polyfluoroamide of a saturated perfluoroaliphatic monocarboxylic acid having from 4 to 22 carbon atoms and an alkyl amine having 8 to 22 carbon atoms in the alkyl chain.

2. A stable, non-foaming petroleum hydrocarbon jet fuel composition consisting essentially of a major amount of a petroleum hydrocarbon jet fuel having a boiling range from about 240° F. to about 600° F. and a Reid Vapor Pressure above 0.5 lb. per sq. in. at 100° F. containing from about 0.01% to about 0.1% by volume of a hydrocarbon-insoluble saturated perfluorocarbon having from 12 to 21 carbon atoms and having a boiling point range of from about 20° C. to about 240° C. at 10 mm. Hg and from about 0.01% to about 10% of a hydrocarbon dispersible polyfluoroamide of an oil-soluble saturated perfluoroaliphatic monocarboxylic acid having from 12 to 18 carbon atoms and an oil-soluble amine having an alkyl radical of from 8 to 22 carbon atoms.

3. A stable, non-foaming petroleum hydrocarbon jet fuel composition consisting essentially of a major amount of a petroleum hydrocarbon jet fuel having a boiling range from about 240° F. to about 600° F. and a Reid Vapor Pressure above 0.5 lb. per sq. in. at 100° F. containing from about 0.01% to about 0.1% by volume of a hydrocarbon-insoluble saturated perfluorocarbon having from 12 to 21 carbon atoms and having a boiling point range of from about 20° C. to about 240° C. at 10 mm. Hg and from about 0.1% to about 10% of a hydrocarbon dispersible polyfluoroamide of an oil-soluble saturated aliphatic monocarboxylic acid having from 12 to 18 carbon

45

atoms and an oil-soluble perfluoroalkylamine the perfluoroalkyl radical having from 8 to 22 carbon atoms.

4. A stable, non-foaming petroleum hydrocarbon jet fuel composition consisting essentially of a major amount of a petroleum hydrocarbon jet fuel having a boiling range from about 240° F. to about 600° F. and a Reid Vapor Pressure of 5-7 lbs. per sq. in. at 100° F. containing from about 0.01% to about 0.1% by volume of an aliphatic perfluorocarbon having at least 21 carbon atoms and a boiling point of at least 130° C. at 10 mm. Hg and from about 0.5% to about 5% of N-C<sub>12-18</sub> alkyl trimethylene fluorocaprylamide.

5. A stable, non-foaming petroleum hydrocarbon jet fuel composition consisting essentially of a major amount of a petroleum hydrocarbon jet fuel having a boiling range from about 240° F. to about 600° F. and a Reid Vapor Pressure of 5-7 lbs. per sq. in. at 100° F. containing from about 0.01% to about 0.1% by volume of a mixture of C<sub>21</sub>F<sub>44</sub> aliphatic perfluorocarbon having a boiling point of 130-240° C. at 10 mm. Hg and C<sub>12</sub>F<sub>26</sub> aliphatic perfluorocarbon having a boiling point of 20-65° C. at 10 mm. Hg in the mole ratio of from 4:1 to 2:1 respectively, and from about 0.5% to about 5% of N-C<sub>12-18</sub> trimethylene fluorocaprylamide.

6. A stable, non-foaming petroleum hydrocarbon jet fuel composition consisting essentially of a major amount of a petroleum hydrocarbon jet fuel having a boiling range from about 240° F. to about 600° F. and a Reid Vapor Pressure of 5-7 lbs. per sq. in. at 100° F. containing from about 0.01% to about 0.1% by volume of a mixture of C<sub>21</sub>F<sub>44</sub> aliphatic perfluorocarbon having a boiling point at 130-240° C. at 10 mm. Hg and C<sub>14</sub>F<sub>30</sub> aliphatic perfluorocarbon having a boiling point of 65-130° C. at 10 mm. Hg in the mole ratio of from 4:1 to 2:1 respectively, and from about 0.5% to about 5% of N-C<sub>12-18</sub> trimethylene fluorocaprylamide.

#### References Cited in the file of this patent

#### UNITED STATES PATENTS

2,394,596 Davis et al. ----- Feb. 12, 1946  
2,680,717 Little ----- Jan. 8, 1954

#### FOREIGN PATENTS

202,976 Australia ----- July 19, 1956